

# United States Patent Office

2,865,741

Patented Dec. 23, 1958

1

2,865,741

## ACID RESISTANT AUSTENITIC STAINLESS STEEL

Raymond Smith, Pittsburgh, Pa., and Charles O. Tarr, Glendale, Ohio, assignors to United States Steel Corporation, a corporation of New Jersey

No Drawing. Continuation of application Serial No. 450,785, August 18, 1954. This application November 6, 1957, Serial No. 694,728

4 Claims. (Cl. 75—125)

This application relates to acid resistant stainless steels and more particularly to forgeable stainless steels that have enhanced resistance to mineral acids such as sulphuric acid.

Stainless steels have heretofore been known which are resistant to corrosive attack by mineral acids. However, such steels have generally been used in cast form since they can only be processed to wrought form by taking severe losses in forging operations or by very special and expensive processing operations which seriously affected the size and shapes that could be so processed.

It is accordingly an object of this invention to provide austenitic stainless steels resistant to mineral acid corrosion which are readily forgeable.

It is a further object of this invention to produce forgeable stainless steels which have a satisfactory resistance to boiling 30% sulphuric acid.

It is another object of this invention to provide acid corrosion resistant stainless steels which are comparatively economical to produce.

According to the teachings of our invention, the foregoing objects can be achieved in steels of the following composition:

|            | Percent      |
|------------|--------------|
| Carbon     | 0.1 to .10   |
| Manganese  | .15 to 2.0   |
| Silicon    | .75 max.     |
| Sulphur    | .04 max.     |
| Phosphorus | .04 max.     |
| Nickel     | 23.0 to 27.0 |
| Chromium   | 17.0 to 20.0 |
| Molybdenum | .80 to 1.5   |
| Copper     | .80 to 1.5   |
| Titanium   | .20 to 2.0   |

We have discovered that the relatively large amounts of silicon, i. e. over 1%, frequently used to obtain enhanced corrosion resistance are very detrimental to forging qualities, whereas with less than about .75% silicon, satisfactory forgeability is obtained. While less than .75% silicon is desirable, it is hard to obtain with present steelmaking techniques. The influence of silicon on forgeability is evident from the following Table I:

Table I

| Heat No. | C   | Mn  | Si   | Ni    | Cr    | Mo   | Cu   | Hot Forgeability |
|----------|-----|-----|------|-------|-------|------|------|------------------|
| 1        | .06 | 1.1 | .45  | 17.56 | 16.86 | .98  | .99  | Satisfactory.    |
| 2        | .06 | 1.0 | .85  | 18.00 | 17.00 | 1.00 | 1.00 | Fair.            |
| 3        | .06 | 1.0 | 1.65 | 18.00 | 17.00 | 1.00 | 1.00 | Unsatisfactory.  |
| 4        | .05 | 1.1 | 2.02 | 18.52 | 15.90 | .95  | 1.08 | Do.              |
| 5        | .20 | 1.0 | 2.00 | 18.00 | 17.00 | 1.00 | 1.00 | Do.              |
| 6        | .06 | 1.0 | 1.77 | 18.00 | 17.00 | 3.00 | 1.00 | Do.              |
| 7        | .06 | 1.1 | 2.12 | 18.52 | 16.40 | 1.04 | 2.82 | Do.              |
| 8        | .06 | 1.2 | 2.00 | 22.00 | 17.00 | 1.00 | 1.00 | Do.              |
| 9        | .06 | .80 | .64  | 22.75 | 16.37 | 1.02 | 1.00 | Satisfactory.    |
| 10       | .07 | 1.4 | .57  | 21.98 | 16.74 | 1.02 | 1.00 | Do.              |

However, lowering the silicon content to develop satis-

2

factory forgeability lowers the corrosion resistance. We have discovered that the corrosion resistance can be restored and even improved by the addition of titanium in amounts over .20% and up to about 2%, particularly if the nickel content is increased slightly. If titanium is added in amounts over 2%, objectionable "stringers" are encountered. The effect of lowering silicon and addition of titanium on corrosion resistance to boiling 30% by weight sulphuric acid is shown in the following Table II. As can be seen reducing silicon increases the corrosion rate to more than .006 I. P. M. (inches penetration per mouth) which is regarded as unsatisfactory.

Table II

| Heat No. | C    | Mn   | Si   | Ni    | Cr    | Mo   | Cu   | Ti  | Corro-<br>sion,<br>I. P. M.<br>Boiling<br>30%<br>H <sub>2</sub> SO <sub>4</sub> |
|----------|------|------|------|-------|-------|------|------|-----|---------------------------------------------------------------------------------|
| 11       | .05  | 1.1  | 2.02 | 18.52 | 15.90 | .95  | 1.08 | —   | .005                                                                            |
| 12       | .06  | 1.0  | 1.65 | 18.00 | 17.00 | 1.00 | 1.00 | —   | .014                                                                            |
| 13       | .06  | 1.0  | .85  | 18.00 | 17.00 | 1.00 | 1.00 | —   | .022                                                                            |
| 14       | .06  | 1.1  | .45  | 17.50 | 16.86 | .98  | .99  | —   | .015                                                                            |
| 15       | .07  | 1.35 | .46  | 23.72 | 16.77 | 1.02 | .98  | —   | .008                                                                            |
| 16       | .06  | 1.30 | .55  | 24.16 | 16.70 | 1.00 | 1.00 | .41 | .004                                                                            |
| 17       | .051 | —    | —    | 24.00 | 17.00 | 1.00 | 1.00 | .15 | .007                                                                            |
| 18       | .049 | —    | —    | 24.00 | 17.00 | 1.00 | 1.00 | —   | —                                                                               |
| 19       | .062 | 1.36 | .60  | 21.96 | 17.04 | .99  | 1.02 | .32 | .005                                                                            |

A comparison of the corrosion data for heats 15, 16, 17 and 18 demonstrates clearly the ability of titanium to lower the corrosion rate to less than .006 I. P. M. This may result from the ability of titanium to scavenge nitrogen and sulphur from the material.

The following Table III demonstrates that substantial resistance to boiling 30% sulphuric acid is obtained with about 1% each of molybdenum and copper when titanium is present.

Table III

| Heat No. | C   | Mn  | Si   | Ni   | Cr   | Mo  | Cu  | Ti  | Corro-<br>sion,<br>I. P. M.<br>Boiling<br>30%<br>H <sub>2</sub> SO <sub>4</sub> |
|----------|-----|-----|------|------|------|-----|-----|-----|---------------------------------------------------------------------------------|
| 20       | .05 | 1.1 | 2.02 | 18.0 | 17.0 | 1.0 | 1.0 | —   | .00515                                                                          |
| 21       | .05 | 1.1 | 1.85 | 18.0 | 17.0 | 2.0 | 2.0 | —   | .00435                                                                          |
| 22       | .05 | 1.3 | .47  | 22.0 | 15.0 | 1.0 | 3.0 | .42 | .00407                                                                          |
| 23       | .06 | 1.5 | .54  | 22.0 | 17.0 | 1.0 | 1.0 | .50 | .00493                                                                          |

However to adequately resist attack in boiling 50% by weight sulphuric acid, i. e. to reduce the I. P. M. to about .01% or less, higher molybdenum is required. This is shown in Table IV.

Table IV

| Heat No. | C    | Mn   | Si  | Ni    | Cr    | Mo   | Cu   | Ti  | Corro-<br>sion,<br>I. P. M.<br>Boiling<br>50%<br>H <sub>2</sub> SO <sub>4</sub> |
|----------|------|------|-----|-------|-------|------|------|-----|---------------------------------------------------------------------------------|
| 24       | .062 | .80  | .64 | 22.75 | 16.87 | 1.02 | 1.00 | .42 | .063                                                                            |
| 25       | .049 | 1.40 | .40 | 21.39 | 16.12 | 2.85 | .98  | .04 | .0103                                                                           |
| 26       | .050 | 1.28 | .51 | 22.00 | 16.88 | 2.95 | 1.02 | .50 | .0083                                                                           |

These higher molybdenum contents contribute to poor hot working characteristics.

Numerous experiments have shown that titanium is unique in respect to enhancing corrosion resistance. The following Table V shows that the elements such as vanadium, columbium, tantalum, tungsten, and zirconium which are sometimes considered equivalents to titanium do not react in the same way as titanium in this respect.

Table V

| Heat No. | C    | Mn   | Si  | Ni    | Cr    | Mo   | Cu   | Others     | Corro-<br>sion,<br>I. P. M.<br>Boiling<br>30%<br>H <sub>2</sub> SO <sub>4</sub> |
|----------|------|------|-----|-------|-------|------|------|------------|---------------------------------------------------------------------------------|
| 27       | .066 | 1.40 | .57 | 21.98 | 16.74 | 1.02 | 1.00 | .37 Ti     | .0055                                                                           |
| 28       | .056 | 1.29 | .59 | 21.82 | 17.11 | 1.03 | 1.00 | .57 V      | .0104                                                                           |
| 29       | .059 | 1.28 | .53 | 22.30 | 17.32 | 1.07 | .98  | 1.01 Cb    | .0084                                                                           |
| 30       | .068 | 1.34 | .54 | 21.20 | 16.90 | 1.03 | .97  | .76 W      | .0107                                                                           |
| 31       | .062 | 1.50 | .63 | 21.20 | 16.72 | 1.03 | .97  | 1.20 Cb+Ta | .0096                                                                           |
| 32       | .059 | 1.38 | .58 | 22.40 | 16.80 | 1.03 | 1.01 | .49 Zr     | .0199                                                                           |

In view of extensive tests, as exemplified by the foregoing tables, we have found that considering the economies of manufacture, the following ranges are preferred:

|            | Percent        |    |
|------------|----------------|----|
| Carbon     | .05 to .08     |    |
| Manganese  | .75 to 1.50    | 20 |
| Silicon    | .60 max.       |    |
| Phosphorus | .04 max.       |    |
| Sulphur    | .04 max.       |    |
| Nickel     | 23.00 to 27.00 |    |
| Chromium   | 17.00 to 20.00 | 25 |
| Molybdenum | .80 to 1.50    |    |
| Copper     | .80 to 1.50    |    |
| Titanium   | .30 to .50     |    |

This application is a continuation of my copending application Serial No. 450,785, filed August 18, 1954, now abandoned.

While we have shown and described several specific embodiments of our invention, it will be understood that these embodiments are merely for the purpose of illustration and description and that various other forms may be devised within the scope of our invention, as defined in the appended claims.

We claim:

1. A readily forgeable austenitic stainless steel highly resistant to corrosion by mineral acids and characterized by an I. P. M. rate of less than .006 in boiling 30% sulphuric acid, said steel consisting of

|            | Percent        |    |
|------------|----------------|----|
| Carbon     | .05 to .08     |    |
| Manganese  | .75 to 1.50    | 43 |
| Silicon    | .60 max.       |    |
| Phosphorus | .04 max.       |    |
| Sulphur    | .04 max.       |    |
| Nickel     | 23.00 to 27.00 |    |
| Chromium   | 17.00 to 20.00 |    |
| Molybdenum | .80 to 1.50    |    |
| Copper     | .80 to 1.50    |    |
| Titanium   | .30 to .50     |    |

with the balance iron and residual amounts of other elements.

2. A readily forgeable austenitic stainless steel highly resistant to corrosion by mineral acids and characterized by an I. P. M. rate of less than .006 in boiling 30% sulphuric acid, said steel consisting of

|            | Percent        |    |
|------------|----------------|----|
| Carbon     | .05 to .08     |    |
| Manganese  | .75 to 1.50    |    |
| Silicon    | .60 max.       |    |
| Phosphorus | .04 max.       | 65 |
| Sulphur    | .04 max.       |    |
| Nickel     | 23.00 to 27.00 |    |
| Chromium   | 17.00 to 20.00 |    |
| Molybdenum | .80 to 1.50    |    |
| Copper     | .80 to 1.50    |    |
| Titanium   | .30 to .50     | 70 |

with the balance iron and other elements in amounts which do not adversely affect the properties.

3. A readily forgeable austenitic stainless steel highly resistant to corrosion by mineral acids and characterized by an I. P. M. rate of less than .006 in boiling 30% sulphuric acid, said steel consisting of

|            | Percent        |
|------------|----------------|
| Carbon     | .01 to .10     |
| Manganese  | .15 to 2.00    |
| Silicon    | .75 max.       |
| Sulphur    | .04 max.       |
| Phosphorus | .04 max.       |
| Nickel     | 23.00 to 27.00 |
| Chromium   | 17.00 to 20.00 |
| Molybdenum | .80 to 1.50    |
| Copper     | .80 to 1.50    |
| Titanium   | .20 to 2.00    |

with the balance iron and residual amounts of other elements.

4. A readily forgeable austenitic stainless steel highly resistant to corrosion by mineral acids and characterized by an I. P. M. rate of less than .006 in boiling 30% sulphuric acid, said steel consisting of

|            | Percent        |
|------------|----------------|
| Carbon     | .01 to .10     |
| Manganese  | .15 to 2.00    |
| Silicon    | .75 max.       |
| Sulphur    | .04 max.       |
| Phosphorus | .04 max.       |
| Nickel     | 23.00 to 27.00 |
| Chromium   | 17.00 to 20.00 |
| Molybdenum | .80 to 1.50    |
| Copper     | .80 to 1.50    |
| Titanium   | .20 to 2.00    |

with the balance iron and other elements in amounts which do not adversely affect the properties.

#### References Cited in the file of this patent

#### UNITED STATES PATENTS

2,506,518 Norris May 2, 1950  
2,553,330 Post May 15, 1951

UNITED STATES PATENT OFFICE  
CERTIFICATE OF CORRECTION

Patent No. 2,865,741

Raymond Smith et al.

December 23, 1958

It is hereby certified that error appears in the printed specification of the above numbered patent requiring correction and that the said Letters Patent should read as corrected below.

Column 1, line 38, for

"Carbon —— 0.1 to .10"

read

— Carbon —— .01 to .10 —;

column 2, line 12, for "mouth" read — month —.

Signed and sealed this 19th day May 1959.

(SEAL)

Attest:

KARL H. AXLINE

Attesting Officer

ROBERT C. WATSON  
Commissioner of Patents